

## UNITED STATES PATENT OFFICE

2,439,901

METHOD FOR PRODUCING COLORED  
PHOTOGRAPHS

Henry T. Neumann, New York, N. Y.

No Drawing. Application December 27, 1941,  
Serial No. 424,574

## 1 Claim. (Cl. 95—2)

**1** This invention relates to a method and means for producing colored photographs.

Heretofore, it has been the practice to either print a plurality of differently colored images on separate emulsion layers which were then superimposed and registered, or to employ special multi-layered emulsions. Both of these methods, however, require the use of relatively expensive, special materials such as stripping emulsions in the first method, and multi-layered emulsions in the second. Furthermore, such methods included many elaborate and delicate procedural steps which consume much time and require a high degree of manipulative and technical skill.

It is an object of my present invention to overcome the difficulties inherent in the foregoing procedures by providing a method which comprises relatively few and simple steps, which may be practiced with good results by persons having only ordinary experience in photography, and which requires no special materials or apparatus.

Another object of my invention is to provide a method of the character described, which may be carried out with standard photographic emulsions.

A further object of my invention is to provide a method of the character described, in which only a single sheet of ordinary emulsion paper is used in printing a colored image.

An additional object of my invention is to provide a method of the character described, in which the several colored components of a colored image are successively printed on a single-layered acromatic emulsion, i. e. an emulsion which is not sensitive to all colors and which does not include a plurality of individual layers so arranged and/or constituted that each layer is photosensitive to a different color.

A supplementary object of my invention is to provide chemical reagents for successfully practicing my novel method.

Other objects of this invention will in part be obvious and in part hereinafter pointed out.

Certain features of the invention described but not claimed herein are described and claimed in my co-pending application for Methods and means for producing a colored photographic image, Serial No. 357,830, filed September 23, 1940; now Patent No. 2,417,514.

In general, I practice my invention by successively forming a series of monochromatic component images of a multichromatic picture in a photosensitive emulsion. The particular monochromatic component colors employed may con-

**2** form with any well accepted practice and are so selected as to render a faithful colored image of the picture being reproduced. After each monochromatic component image has actinically effected the photosensitive emulsion, and before the next monochromatic colored image is projected, the emulsion is developed to bring out a colored picture corresponding to the monochromatic component image cast. If necessary or desirable, the emulsion is treated after each but the last color development to "set" or prevent the developed color image from being affected by any subsequent steps in my process and particularly by any subsequent steps in developing further colors. Since this last step tends to reduce the photosensitivity of the silver salts, I preferably treat the emulsion after or during such setting step to offset such decreased sensitivity and to substantially or partially restore said emulsion to its original state of photosensitivity. All of the monochromatic component images are projected in registry upon the same single photosensitive emulsion. In developing the latent images formed in the photosensitive emulsion, any suitable method for developing colors may be employed. The emulsion is not exposed to actinic rays, except when modulated by color component images, until all the colors have been developed. It will thus be apparent that after all of the monochromatic component images, such as for example blue, red and yellow, have been separately projected upon and developed in the photosensitive emulsion, the original colored picture will be exactly reproduced in full color in the single layer of photosensitive emulsion.

I prefer to carry out my invention by using a dye-coupling developing process, such as described in my aforesaid copending application, and when such method of color developing is employed, the following steps, in general, are performed:

First, black and white color separation negatives are made in the usual manner from a colored picture or transparency, as by employing colored filters. After preparing such negatives, an actinic printing light is passed through one of the negatives, for example, the blue one, and projected upon the surface of the photosensitive emulsion. The exposure of the photosensitive emulsion may be performed in any standard apparatus, such as for example an enlarger or a contact printer. When black and white color separation negatives are employed with the usual white printing light, either achromatic or pan-chromatic emulsions may be used. However, I

prefer achromatic emulsions, since red light may then be present in the developing room and the course of the development closely observed. If panchromatic emulsions are used, color separation negatives may be dispensed with, and in lieu thereof monochromatic beams of light successively reflected from or passed through the colored picture to be reproduced and then projected upon the emulsion. The monochromatic beams employed may correspond to the monochromatic component colors used to form the color separation negatives. When panchromatic emulsions are employed, all treatments subsequent to formation of latent images are similar to the treatments of achromatic emulsions.

After a latent image corresponding to a component color of the picture being reproduced has been formed in the photosensitive emulsion, said image is developed by reduction. A standard non-coupling developing agent may be used, such as for example "metol," whose properties in connection with color developing by dye-coupling are fully set forth in my copending application. While the image is being reduced, it is simultaneously treated with a coupling-inducer, which may be of a reducing nature, and a color-coupler which corresponds to the color component of the first or blue negative separation image. Any standard coupling-inducers and color-couplers well known to the art may be employed in the process herein described.

Since the same photosensitive emulsion is to be treated in several reducing and coupling baths, I preferably employ means to prevent too great a softening of the emulsion and also to prevent fogging, which might be incident to treatment in three separate developing baths. The anti-softening or hardening reagent employed may be any suitable gelatin-hardening substance, as for example an alkali metal sulphate. In conjunction with the hardening reagent, it is also desirable to use a strong accelerating agent in the developing bath. An example of such an accelerating agent is sodium hydroxide. The combination of a strong accelerator and a hardener I have found prevents staining of the clear portions of the film and prevents too great a softening of the gelatin emulsion.

Owing to the fact that after one color has been coupled the emulsion is, at a later stage hereinafter described, treated with other color couplers which may affect the first coupler color, I have found it desirable to treat the first developed monochromatic image in a bath to "set" the developed image, i. e. to disturb the capacity of the formed color to unite with other color couplers or chemicals used in subsequent steps of my process. Various chemical reagents have been found to be satisfactory for this purpose. Examples of these reagents are alums, such as chrome alum or potassium alum, formaldehyde, paraformaldehyde, sodium acid sulphite, tartaric acid, citric acid, tannic acid, and sodium formate. These setting reagents can be used independently or in combination, and highly satisfactory results have been obtained when sodium formate is used with one or more of the other reagents.

If desired, there may also be employed standard salting reagents in the setting solution to better precipitate the colors. These reagents, however, must not affect the photosensitive silver salts. By way of example, such reagents may comprise sodium carbonate, ammonium sulphate, sodium phosphate, calcium acetate, and hexa-

methylenetetramine. Where the salting reagent is alkaline in nature, as for example in the case of sodium carbonate, it is desirable to add a mild or very dilute acid or an acid salt, as for example phosphoric acid, citric acid, tartaric acid, dilute acetic acid (one part in ten thousand) or sodium acid phosphate. These acidifying reagents reverse the alkalinity of the emulsion caused by the developing bath. It will be appreciated that the standard salting reagents are always used with a reagent for hardening the gelatin or with a reagent which will react with the salting reagent to produce a compound which will harden the gelatin. Examples of such hardening reagents, which, it will be seen, include some of the setting reagents above set forth, comprise formaldehyde, alums such as chrome alum or potassium alum, paraformaldehyde, tannic acid, sodium sulphate, magnesium sulphate, and phthalic anhydride. In the foregoing list, the phthalic anhydride represents an example of a compound which will react with the salting reagent, hexamethylenetetramine to produce or free a substance, formaldehyde, for hardening the gelatin emulsion.

It will thus be seen that the bath in which the emulsion is treated subsequent to the first developing preferably contains reagents to perform the following functions: setting, salting, acidifying and hardening. However, it is not necessary to have a separate reagent for each of these stated functions, as one reagent may serve to perform two or more such functions.

The setting and hardening reagents tend to decrease the sensitivity of the emulsion towards future exposures, and to offset such desensitization I may provide a reagent which inhibits the desensitizing effect of the setting reagent or which resensitizes the emulsion. An example of a reagent which offsets the effect of the setting reagent is potassium ferrocyanide. This latter reagent greatly decreases the exposure time required to form latent images of color separation negatives subsequent to development of the first color separation image. It may be noted that where a chrome alum and sodium formate setting bath is employed, the time of exposure for the next negative is twenty times as great as when no such setting bath is employed. But if after treatment with such setting bath, I submerge the emulsion in a ferrocyanide bath, the time of exposure required for future negatives is considerably reduced.

Other examples of desensitizing-inhibiting or resensitizing reagents comprise certain salting reagents, including the halide salts of metals or positive radicals which do not detrimentally affect the photosensitive silver halides. Examples of such salting reagents are ammonium, lithium, strontium and nickel halides. The halides which I preferably use are bromides and chlorides, although other halides may be employed to attain certain color effects not ordinarily desired. I have found the halides restore the sensitivity of the "set" emulsion to a much greater degree than the ferrocyanide, and the emulsion by such treatment may be rendered even more sensitive than before exposure.

It may be mentioned that the desensitizing or resensitizing reagent may be present either in the setting bath or in a separate bath, although I prefer to place such reagent in the setting bath.

After the first or blue monochromatic colored image is set, the emulsion is washed. It is then

placed in the enlarger or contact printer in the same position that it occupied during the first exposure, and exposed to a printing light modulated by a second color separation negative, for example red. The red separation negative occupies exactly the same position as the first or blue separation negative. This exposure will cause the formation of a second latent image in the emulsion. Said image is reduced and coupled to bring out a monochromatic picture corresponding in color to the color of the second separation negative. This second picture is set and the emulsion treated in a sensitizing or desensitization-inhibiting bath. After washing, the emulsion is returned for printing with a third or yellow separation negative. The latent image formed is developed and coupled to bring out the third color component which does not have to be set since no further developing treatments are to be performed upon the emulsion.

At this time, the emulsion, if properly exposed and developed in connection with each of the three colors, presents a faithfully colored reproduction of the original image; and the emulsion can now be stopped in a hypo solution. If the emulsion is to be used as a motion picture positive, the process may be halted at this stage. If, however, the emulsion is to be used as a positive print on paper, it is also desirable to bleach out the reduced silver grains. This is accomplished by treatment in the usual bleaching baths of the art.

I have found it desirable to first expose the emulsion to a blue separation negative, then to a red separation negative and finally to a yellow separation negative. This order of exposure and development is particularly effective where an achromatic photo sensitive emulsion is employed.

It may be mentioned that after the yellow color development, the reproduction may be examined for yellow color tone value and that the yellow may be varied in intensity if necessary before stopping the emulsion in hypo.

By way of example, I have set forth below various specific chemicals and procedural steps which are employed in carrying out my invention. These chemicals and steps have been found to give highly satisfactory results. It is to be understood, however, that the examples are in no way to be considered limitative.

#### Example I

First, blue, red and yellow separation images of the picture to be produced are prepared. The blue separation negative is then placed in position in an enlarger. A sheet of ordinary achromatic silver halide printing paper is wetted, as for example in water, and then also placed in the enlarger, the negatives and printing paper being positioned in the usual manner so that a beam of white printing light modulated by the blue negative will be projected upon the paper. The wetting step is performed in order to swell the paper fibres, thereby placing the paper in the same condition that it will be in during subsequent printing steps and ensuring registration. The source of light in the enlarger is now energized and the paper exposed for a sufficient period of time to form a latent image therein. This period of exposure will vary with the type of printing paper employed and with the density of the picture to be reproduced. For convenience, the blue exposure period will be denominated as one unit of exposure value.

After exposure, the paper, having the latent blue component image therein, is developed in a bath prepared according to the following instructions:

5 The developing bath is formed by mixing together several stock solutions. Stock solution A is prepared from a dry powder including the following substances in the specified proportions by weight:

|                        | Grams |
|------------------------|-------|
| 2-4 dichloro-1 naphtol | 4     |
| Sodium sulphite        | 10    |
| Sodium acid phosphate  | 1     |

10 One gram of the dry powder is dissolved in 15 cc. of acetone and 50 cc. of water. Such a stock solution is good for approximately one week.

Stock solution B is prepared from a dry powder including the following substances in the specified proportions by weight:

|                                             | Grams |
|---------------------------------------------|-------|
| Para - aminodiethylanalinemonohydrochloride | 3     |
| "Metol"                                     | 1     |
| Sodium sulphite                             | 15    |

15 One gram of the dry powder is dissolved in 50 cc. of water. This stock solution will last indefinitely.

Stock solution C is prepared from a dry powder including the following substances in the specified proportions by weight:

|                  | Grams |
|------------------|-------|
| Sodium borate    | 6     |
| Sodium sulphite  | 4     |
| Sodium hydroxide | 40    |

20 One gram of the dry powder is dissolved in 50 cc. of water. This stock solution will last indefinitely.

Stock solution D is prepared from a dry powder including the following substances in the specified proportions by weight:

|                        | grams |
|------------------------|-------|
| Sodium formate         | 4     |
| Potassium ferrocyanide | 1     |

25 Five grams of the dry powder is dissolved in 100 cc. of water. This stock solution will last indefinitely.

55 The sodium formate and potassium ferrocyanide in the dry powder are not merely mixed together, but these substances are dissolved and subsequently recrystallized so as to increase the solubility of the ferrocyanide and thereby render the process more easily practiced by amateurs.

The developing solution is prepared by mixing together:

|                  |    |     |
|------------------|----|-----|
| Stock solution A | cc | 10  |
| Stock solution B | cc | 20  |
| Stock solution C | cc | 20  |
| Stock solution D | cc | 10  |
| Water            | cc | 150 |

60 Ten percent water solution of potassium bromide

drops 2

65 For developing in this solution, the bath is maintained at a temperature of from about 65 to 68° F. The developing will require from three to five minutes, although the image will appear in between thirty to fifty seconds.

70 The sheet is now washed in running water for about one minute. Next, the sheet is immersed in a setting solution wherein it is moved around for about one minute. The temperature of the

setting solution is maintained at about 65 to 68° F. The setting solution is prepared by mixing together:

|                                               |    |    |
|-----------------------------------------------|----|----|
| 5 percent of water solution of chrome alum    | cc | 50 |
| 5 percent of water solution of sodium formate | cc | 60 |
| Stock solution D                              | cc | 10 |

The next step comprises washing the sheet in running water from three to five minutes. Finally, the sheet is squeegeed.

The damp sheet is then returned to the enlarger and exposed to a printing light modulated by the red separation negative for a period of time substantially equal to four units of exposure value to form a red component latent image in the emulsion. This image is developed by immersing the sheet in a red coupling and developing bath prepared as follows:

A stock solution E is made from a dry powder including the following substances in the specified proportions by weight:

|                              |       |   |
|------------------------------|-------|---|
| Para-nitrophenylacetonitrile | grams | 1 |
| Sodium acid phosphate        | grams | 1 |
| Sodium sulphite              | grams | 5 |

One gram of the dry powder is dissolved in 15 cc. of acetone and 50 cc. of water. This solution is good for about one week. The red developing solution is similar to the blue developing solution, except that 10 cc. of solution E is substituted for 10 cc. of solution A.

The duration of developing and the temperature of the red developing bath are the same as when developing the blue component image. After developing, the sheet is washed, set, washed and squeegeed as described with reference to the blue image.

Now the sheet is again replaced in the enlarger and this time exposed to a printing light modulated by the yellow separation negative. The printing time for the yellow negative is twelve units of exposure value. The yellow component latent image thus formed on the sheet is developed in the same manner as the red and blue images. However, 10 cc. of stock solution F replaces solutions A and E.

Said stock solution F is prepared from a dry powder including the following substances in the specified proportions by weight:

|                           |       |   |
|---------------------------|-------|---|
| Aceto 2-5 dichloroaniline | grams | 6 |
| Sodium sulphite           | grams | 4 |
| Sodium acid phosphate     | grams | 1 |

One gram of the dry powder is dissolved in 15 cc. of acetone and 50 cc. of water. This solution will last for long periods of time.

The sheet is now washed in running water for one minute, but the treatment in the setting bath is omitted.

The sheet is next desensitized in a hypo bath. For this purpose, the sheet is immersed in the hypo bath for two minutes while the bath is maintained at a temperature of from about 65 to 68° F. The hypo bath is the standard one prepared by adding two pounds of sodium hyposulphite and five grams of sodium bisulphite to one gallon of water.

While the print is still wet with hypo solution, it is immersed in a bleaching bath to remove the reduced silver grains. The bleaching bath is a one per cent water solution of potassium ferricyanide. The print is left in the bleaching bath

for from 45 seconds to 2 minutes while the bath is maintained at a temperature of from about 65 to 68° F. This bath will remove all reduced silver.

The yellowish stain left by the ferricyanide bath is removed by returning the print to the hypo bath and leaving same there for about one minute.

Finally the print is washed in running water for from five to eight minutes, squeegeed for finish and dried.

#### Example II

When it is desired to employ halide salts in the setting bath, I may substitute for the setting bath described in Example I a bath made up as follows:

15 Stock solution G is prepared from a dry powder including the following substances in the specified proportions by weight:

|                |       |    |
|----------------|-------|----|
| Potassium alum | grams | 25 |
| Sodium formate | grams | 25 |

Fifty grams of the dry powder is dissolved in 1,000 cc. of water. This solution will last indefinitely.

Stock solution H is prepared by adding five grams of ammonium bromide to 100 cc. of water. This solution will also last indefinitely.

100 cc. of stock solution G is mixed with 10 cc. of stock solution H to form a setting bath which also includes a silver halide sensitizing reagent. When halides are employed in a setting bath, the red separation negative needs only to be exposed for one and one-half units of exposure value and the yellow separation negative for three units of exposure value.

30 The emulsion sheet is left for about one and one-half minutes in the above bath which is maintained at a temperature of from about 65 to 68° F.

#### Example III

40 Where it is desired to employ a salting reagent which reacts with another compound to produce a hardening reagent in the setting bath, the following solution may be employed in lieu of the setting solution given in Example I:

45 Solution I is prepared by dissolving two grams of phthalic anhydride in 100 cc. of boiling water. While the water is still hot, five grams of hexamethylenetetramine is added. The solution is now allowed to cool and another 100 cc. of water is added. This solution will last indefinitely.

50 Solution J is prepared from a dry powder including the following substances in the specified proportions by weight:

|                   |       |   |
|-------------------|-------|---|
| Ammonium bromide  | grams | 5 |
| Ammonium chloride | grams | 5 |

55 Five grams of the dry powder is dissolved in 100 cc. of water. This solution will last indefinitely.

100 cc. of solution I is added to 20 cc. of solution J to form a setting bath. It will be noted that this bath includes a halide reagent. The bath is used at a temperature of from about 65 to 68° F. at which the emulsion is treated for about one to one and one-half minutes.

60 It will thus be seen that there is provided methods and means by which the several objects of this invention are achieved, and which are well adapted to meet the conditions of practical use.

70 As various possible embodiments might be made of the above invention, and as various changes might be made in the embodiments above set forth, it is to be understood that all matter herein set forth is to be interpreted as illustrative and not in a limiting sense.

Having thus described my invention, I claim as new and desire to secure by Letters Patent:

A method of producing a colored photograph of a multichromatic picture in a single-layered emulsion having photosensitive particles distributed throughout, comprising successively forming registered latent images of different monochromatic components of said picture in said emulsion by successively casting on one side thereof beams of light modulated by different color components of said picture and, prior to forming each latent image, subsequent to the first latent image, color developing the preceding latent image by dye-coupling, disturbing the capacity of the coupled dye to unite with chemicals subsequently used for forming other coupled dyes without affecting any previously actinically affected photosensitive particles, and offsetting the decreased photosensitivity of said photosensitive particles resulting from such disturbance, said disturbance and offsetting of the decreased photosensitivity being effected by treating the emulsion in a bath including hexamethylene-tetramine, phthalic anhydride and a halide.

HENRY T. NEUMANN.

#### REFERENCES CITED

The following references are of record in the file of this patent:

#### UNITED STATES PATENTS

|    | Number    | Name            | Date          |
|----|-----------|-----------------|---------------|
| 10 | 1,207,527 | Fox             | Dec. 5, 1916  |
|    | 1,710,455 | Langguth et al. | Apr. 23, 1929 |
|    | 1,963,197 | Froehlich       | June 19, 1934 |
|    | 1,968,956 | Murray et al.   | Aug. 7, 1934  |
|    | 1,976,301 | Seymour et al.  | Oct. 9, 1934  |
|    | 2,059,887 | Mannes et al.   | Nov. 3, 1936  |
|    | 2,151,532 | Schmidt et al.  | Mar. 21, 1939 |
| 15 | 2,198,827 | Leuch           | Apr. 30, 1940 |
|    | 2,200,018 | Bertrand        | May 7, 1940   |
|    | 2,244,589 | Yanket          | June 3, 1941  |

#### FOREIGN PATENTS

|    | Number  | Country       | Date          |
|----|---------|---------------|---------------|
| 20 | 404,856 | Great Britain | Jan. 25, 1934 |